

106  
1/9

(No Specimens.)

M. P. HAYES.

PROCESS OF CASTING METALS.

No. 317,533.

Patented May 12, 1885.



Attest:  
H. J. Barnhard  
F. C. Reeside

Inventor:  
Martin P. Hayes  
By his Attorneys  
Edson Bros.

X R

## UNITED STATES PATENT OFFICE.

MARTIN P. HAYES, OF CHICAGO, ILLINOIS, ASSIGNOR OF ONE-HALF TO FREDERIC ERIC MORTIMER ATKINSON, OF SAME PLACE.

## PROCESS OF CASTING METALS.

SPECIFICATION forming part of Letters Patent No. 317,533, dated May 12, 1885.

Application filed November 3, 1884. (No specimens.)

22-211

*To all whom it may concern:*

Be it known that I, MARTIN P. HAYES, a citizen of Great Britain, residing at Chicago, in the county of Cook and State of Illinois, have invented certain new and useful Improvements in Processes of Casting Metals, of which the following is a specification, reference being had therein to the accompanying drawings.

My invention relates to a method of casting metal articles; and the novelty consists in the manner of carrying out the same, as will be fully hereinafter described, and specifically pointed out in the claims.

In casting as heretofore practiced it has been a desideratum to obtain a metal as free as possible from crystallization and "blow-holes." These features are caused by the motion of heat from the molten body of metal in the direction of the nearest cooler surfaces, affecting the atoms of metal to vibratory motion, and the presence of air in the molds causes an evolution of gases, which causes blow-holes in the casting. When the metal becomes cooled, this crystallization causes weak brittle castings. It is my design to prevent this crystallization, and to this end I propose to cool very slowly to prevent the travel of heat from vibrating or giving motion to the atoms of metal until it reaches a plastic consistence, in which state the atoms are not so liable to motion from this cause, and in which crystallization is not liable to occur to the same extent as in ordinary casting. With this same object in view various attempts have been made to produce superior castings, and molds have been made of such refractory material that they have been susceptible of being raised to a high temperature. In the attempt to produce a better quality of metal the same has been cast *in vacuo*, the molds being made air-tight and the air exhausted at some period during the process of filling.

With these worthy attempts in view the object of my invention may be said to be to prevent crystallization and to produce a more perfect casting at a minimum cost.

I prevent crystallization by raising the temperature of the metal when it is poured into the molds to, say, 2,300° Fahrenheit. This temperature I retain through the mold for a considerable time after the metal is poured in, and this prevents any considerable current of

heat from the center of the metal toward a cooler portion. The degree of heat is very gradually lessened until the metal assumes a pasty condition and the atoms or molecules no longer possess the freedom of motion which is necessary for perfect crystallization. By the exclusion of air and the keeping of the metal at a high temperature in the molds for some time after it is poured in, I prevent the evolution of gases and the formation of crystals, thus producing what is called in the trade a "solid casting." I, in other words, attain such a condition that no change takes place in the state of the metal when it is placed in the molds, and then so retard the cooling that the metal has assumed a pasty condition before a sufficient force has developed by radiation of heat to cause crystallization. In order to attain this condition, I employ molds made entirely of refractory material—such as fire-clay or mixture of fire-clay and plumbago—and I polish the insides of the molds with a thin coating of plumbago and sour beer. These molds are made sufficiently stout to resist the pressure of the metal by their own strength and without the aid of other metal or casings or flasks, which would interfere with the application of great heat to the exterior surfaces. The molds are formed, dried, and baked in two or more parts, and these parts are brought together and cemented properly to each other to make air-tight joints. This joint may be made with a luting of silicate of soda, fire-clay, fine linseed-meal, and water or sour beer. Each mold complete is made with two pipe-connections, one to be connected with an air-pump and the other with a pipe for admitting the molten metal.

In casting tires or blooms for making locomotive-tires, for instance, I provide a series or stack of furnaces. As an example of the means for carrying my process into practical use, I append hereto a set of illustrations, in which—

Figure 1 shows an exterior view of a furnace and a set of molds therein having their connections made with an exhausting apparatus and source of metal supply. Fig. 2 is an internal sectional view of such furnace, showing tuyeres for an injection of a blast to produce an intense heat. Fig. 3 represents sectional views of a tire-mold.

In the drawings, in which like letters of ref-

erence denote like parts, M designates the mold; A, the furnace; D, the doors thereof, and Q the tuyeres for the injection of a blast to produce intense heat to the interior; B, the smoke-stack; E, the exhaust-connection, and P the connection with a source of molten metal, these latter pipes, E and P, being provided with proper cocks and valves *e p*, respectively.

The furnaces, but one of which is shown, being prepared and charged with a proper layer of coke, and the molds prepared and placed in position, and the air-pipes and metal-supply pipes connected, and the joints in the molds luted, the fires are started. When the molds have reached a white heat, the air is withdrawn from the interior of the molds, and the stop-cocks *e* in the air-pipes E are then closed, care having been taken to have the molds reach a heat corresponding to that of the molten metal, and the metal admitted to the mold in sufficient quantity through the pipes P, the valve of which is then closed to cut off the supply of metal. By means of the tuyeres the heat can be properly adjusted to allow the molds to cool very slowly—say ten to fifteen days; but I would have it understood that the time for cooling will vary with the weight and shape of the castings. The molds are then removed and separated carefully to allow their reuse.

This invention must not be confounded with simple casting *in vacuo*, nor simple slow cooling. It consists in a succession of steps and conditions, which combined go to make a novel and successful method for the purpose described.

What I claim as new is—

1. The process herein described of casting metal, which consists in first subjecting in a furnace air-tight molds made entirely of refractory material to a heat approximating that of the molten metal to be cast, then exhausting the air and introducing the molten metal, and finally slowly reducing the temperature of the furnace, as set forth.

2. The process of casting described, which consists of subjecting molds of refractory material joined with a luting to heat in a furnace, raising the temperature of said molds to a point corresponding to that of the molten metal, exhausting the air from the air-tight molds and introducing the molten metal therein, and slowly reducing the heat of the furnace, as set forth.

In testimony whereof I affix my signature in presence of two witnesses.

MARTIN P. HAYES.

Witnesses:

JAMES A. MAIN,  
E. O. MCNAIR.